

Jan. 24, 1928.

1,656,901

R. F. BUCHHOLZ

RESISTANCE ELEMENT

Filed June 24. 1924



Fig. 1.



Fig. 2.

RENE F. BUCHHOLZ *INVENTOR*  
BY *Cornelius L. Ehret*  
*his ATTORNEY*

Patented Jan. 24, 1928.

1,656,901

## UNITED STATES PATENT OFFICE.

RENÉ F. BUCHHOLZ, OF PHILADELPHIA, PENNSYLVANIA, ASSIGNOR TO ATWATER KENT MANUFACTURING COMPANY, OF PHILADELPHIA, PENNSYLVANIA, A CORPORATION OF PENNSYLVANIA.

### RESISTANCE ELEMENT.

Application filed June 24, 1924. Serial No. 721,964.

My invention relates to resistances, and more particularly to resistances utilizable in connection with audions and similar devices for affording leakage paths or for coupling the output circuit to another circuit.

In accordance with my invention the resistance material comprises lead oxide, preferably litharge, and glycerine or equivalent, forming therewith a solid having the property of binding or cementing; and more particularly my resistance material comprises a mixture of litharge with lamp black or equivalent finely divided conducting material, and glycerine or equivalent.

For an understanding and illustration of my invention reference is to be had to the accompanying drawing, in which:

Fig. 1 is a longitudinal sectional view of a resistance unit in accordance with my invention.

Fig. 2 is a diagrammatic view illustrating one of the various uses of my resistance unit.

Referring to Fig. 1 there is shown disposed within the bore of the tube 1, of glass or other suitable material, a mass 2 of resistance material whose ends are continuous with or homogeneously united with masses 3 of the same or other suitable material disposed within the cap or ferrule members 4 of brass or other suitable conducting material suitably secured or cemented to the tube 1 by material 5 which may be the same as the material 2 or 3, or may be any other suitable material, the masses 3 effecting electrical connection between the mass 2 and the ferrules 4, and the material 5 serving not only as a cement but serving also when of suitable composition to make further electrical connection with the ferrules 4.

The material 2 comprises lead oxide, preferably litharge, mixed in suitable proportion with glycerine, as in forming the well known litharge binder or cement. This material when solidified or hardened, either by application of suitable elevated temperature for suitable time or when subjected to ordinary atmospheric temperature for a longer time, has a high specific resistance, as of the order of 6 megohms per centimeter cube. This material may be disposed in a mass of such length and cross section as to effect a

desired high resistance, as of the order of 1 to 4 megohms when to be utilized as a grid leak resistance or in similar relation.

By preference however I prefer that the resistance material shall have lower specific resistance, particularly for the purpose of rendering it suitable for use in relatively smaller masses of dimensions suitable for the formation of a resistance unit which will fit definitely dimensioned terminal structures or mountings, especially those commonly used in connection with audion or like tubes.

For this purpose there is admixed with the lead oxide, preferably litharge, and preferably before application of the glycerine or equivalent, lamp black or suitably finely divided graphite, carbon, metal or other conducting material. There may be added to 300 grams of pulverized litharge 1.2 grams of lamp black and after thorough mixture there are admixed 2 fluid ounces of glycerine or equivalent.

A mixture of this character when hardened or solidified will have a specific resistance of the order of .8 to 1 megohm per centimeter cube. The mass 2, Fig. 1, of this composition having a diameter of  $\frac{5}{8}$  of an inch and a length of  $1\frac{7}{16}$  inches will have a resistance of the order of 3 megohms.

When a similar mixture comprises about 300 grams of litharge to 1.7 grams of lamp black, with admixture of about 2 fluid ounces of glycerine or equivalent, it will have after baking or hardening a resistance of about  $1\frac{1}{4}$  megohms when of the aforesaid dimensions, namely  $\frac{5}{8}$  of an inch diameter and a length of  $1\frac{7}{16}$  inches; and has a specific resistance of about .3 megohm per centimeter cube.

A mixture of 300 grams of litharge and  $\frac{3}{4}$  of a gram of lamp black and about 2 fluid ounces of glycerine will effect a unit of the aforesaid dimensions having a resistance of about  $4\frac{1}{2}$  megohms; the specific resistance of this mixture is about 1.2 megohms per centimeter cube.

And so on, various other resistances may be obtained by suitably proportioning the lamp black to litharge.

In general I prefer to use a mixture of

the character described having a specific resistance ranging from about .1 to about 2 megohms per centimeter cube. It will be understood that with respect to other aspects of my invention any suitable specific resistance is comprehended.

After the preparation of the mixture of litharge, lamp black or equivalent and glycerine or equivalent it is disposed in suitable 10 form or shape and then hardened as by subjection to ordinary atmospheric temperature for a period of about twenty-four hours or by baking at about 200° F. for about one hour.

15 The units of the character shown in Fig. 1 may be formed by cutting a tube into suitably short lengths to form the tube 1 of Fig. 1 and the material then introduced in the plastic state, and while still plastic the 20 ferrules 4 are applied, suitable amounts of the same mixture, or any equivalent or suitable material, having been first introduced into the ferrules to make intimate contact or become continuous with the material 25 and to afford the masses 5 for holding the ferrules on the tube 1. The material 5 is preferably of a cementitious character and for this purpose may be of the same composition as the mass 2.

30 After so introducing the plastic material and applying the ferrule, the structure is subjected to atmospheric or higher temperatures for the times above indicated whereupon the material solidifies or hardens, 35 without material or substantial adhesion to the glass tube 1, but cementing or adhering or binding to the metal ferrules 4.

A preferred method of introduction is to 40 force the plastic material 2 under pressure into a long glass or similar tube, and while the material therein is still plastic cutting it into suitable lengths, such as the lengths 1, Fig. 1, and then there is applied to each such length the ferrules 4 or equivalent terminals, as above described, and the baking or hardening is thereafter effected.

The resistance material of the character described has the advantage that different 50 resistance units will correspond suitably closely in resistance. Furthermore this material utilized as a grid leak or in similar relation is noiseless, in the sense that there do not occur therewith the audion or tube noises commonly experienced with grid 55 leaks comprising pencil marks, graphitized paper and the like.

The composition described furthermore is 60 of a character which does not absorb moisture to substantial degree and at any rate does not absorb moisture sufficient to materially alter its resistance or to affect its behavior in use, and it is therefore indifferent to changes of humidity and similar atmospheric conditions.

65 The composition, structure and method

described lend themselves to cheap and rapid production of resistance units. The litharge and lamp black or equivalent are intimately and thoroughly mixed by mixing machinery and then after admixture 70 with suitable amount of glycerine or equivalent, is forced as described, into long glass or similar tubes which are then cut into desired lengths while the composition or mixture is plastic and the ferrules or terminals 75 then applied to individual lengths.

Referring to Fig. 2 there is shown a typical radio receiving apparatus comprising an audion or similar thermionic vacuum tube V utilized as a detector. The tube comprises 80 an anode a, grid g and filament or cathode f. In circuit with the grid is the usual grid condenser K in shunt to which is connected the grid leak resistance unit of the character described. As indicated the ferrules 4 are 85 received in and connect with the terminal supports or mountings 6, 6, which are connected to opposite sides of the condenser K. In the anode circuit is the usual battery B and telephone or equivalent device T. The 90 grid circuit contains as usual the tuning condenser C in shunt to the secondary S coupled to the primary P connected with the condenser C' between the antenna A and earth E.

95 It will be understood that a resistance unit of the character described may also be connected directly from the grid g to the filament f, or may be connected between any two electrodes of an audion or similar vacuum tube. It may also be used in the anode circuit of an audion to effect a coupling with another circuit, which may be for example the grid circuit of a second stage tube.

In a material of the character hereinbefore 105 describe the litharge and glycerine apparently re-act upon each other chemically to produce among other things organic compounds of lead, the product having cement-like characteristics which are of advantage 110 in effecting good and permanent electrical connection between the resistance material and a terminal.

What I claim is:

1. An electrical resistance comprising finely divided carbon distributed through a product of mixture of lead oxide with glycerine.

2. An electrical resistance comprising finely divided carbon distributed through a product of mixture of litharge and glycerine.

3. An electrical resistance comprising lamp black distributed through a product of mixture of lead oxide with glycerine.

4. An electrical resistance comprising lamp black distributed through a product of mixture of litharge and glycerine.

5. A resistance material comprising finely divided conducting material distributed 130

through the product of mixture of litharge and glycerine, the proportions to each other of the finely divided conducting material and litharge being such as to effect a specific resistance from about .1 to about 2 megohms per centimeter cube.

6. A resistance material comprising lamp

black distributed through a product of mixture of litharge with glycerine, the proportions to each other of lamp black and litharge being such as to effect a specific resistance of from about .1 to about 2 megohms per centimeter cube.

RENÉ F. BUCHHOLZ.